

## UNITED STATES PATENT OFFICE

1,970,268

METHOD AND MEANS FOR BRIGHT FINISH-  
ING METALS

Arthur E. Bellis, Branford, Conn.

No Drawing. Application August 17, 1932  
Serial No. 629,238

12 Claims. (Cl. 148—8)

This invention relates to an improved method and means for bright finishing metals. It has for its object the removing of surface blemishes from metal and to completely remove all scale, oxide or other surface blemishes thereon, and to provide the metal with a bright finish or lustrous surface protected against corrosion or tarnishing. It has also for its object to treat bright metal and to maintain it in that condition.

10 In carrying out my invention, as one feature thereof, I employ an ammonium formate solution as a quenching bath for the heat-treated metal, as a hot washing liquor, or as a cold soaking bath. I have found that this solution if maintained 15 near its boiling temperature will act very quickly to completely dissolve all scale or oxides and remove heat treatment blemishes from the surface of the metal, while the use of the cold solution and a long soaking treatment of the metal therein, provides the metal surface with a very 20 lustrous finish.

Also, in carrying out the invention, a metal which has its natural bright finish may be treated 25 by the ammonium formate solution, either hot or cold, as described, and the wet solution or the residue after the volatile components of the solution have evaporated, adhering to the metal, have a greater affinity for oxygen than has the metal, so that the metal does not tarnish.

30 Also the particular composition of this ammonium formate solution constitutes an important feature of my invention.

With the above and other objects in view, the invention will be hereinafter more fully described 35 in detail in a preferred embodiment thereof and subsequently defined in the appended claims.

In the practical development and use of my present invention, more particularly in relation 40 to its efficacy in the removal of scale, oxides and other surface blemishes from heat-treated metals, I have found that it is quite immaterial what the particular heat-treating medium or equipment may be. However, best results may be obtained in the use of the present invention by 45 heat-treating the metal in a highly liquid salt bath, and preferably such a bath which has the characteristics of a eutectic. It is also to be understood, that my present invention may likewise be used to advantage in providing the desired 50 bright surface finish upon tarnished cold metal not subjected to such heat treatment. I have found this solution to be highly effective in completely removing all scale, oxide or other surface blemishes which may have been acquired by 55 the metal in the process of heat-treatment so

that when the metal is removed from such solution, it will possess an absolutely clean and bright surface of virgin metal finish. This scavenging action will take place very quickly, if the solution is maintained at a temperature near its 60 boiling point.

When metal having a bright finish, that is, untarnished, is treated, it is subjected to either the hot or cold ammonium formate solution.

In the practice of my invention, I first form 65 an ammonium formate solution or bath. This bath may be most conveniently and inexpensively prepared by dissolving ammonium carbonate and sodium formate in approximately equal proportions in water. As a suitable mixture, I use in 70 each one hundred pounds of water, substantially four and one-tenth pounds ammonium carbonate,  $(\text{NH}_4)_2\text{CO}_3$ , and five and nine-tenths pounds of sodium formate,  $2\text{HCOONa}$ . These chemical components combine to form sodium 75 carbonate,  $\text{Na}_2\text{CO}_3$  and ammonium formate,  $2\text{HCOONH}_4$ . The resulting solution has a slightly alkaline reaction.

The ammonium formate solution above described may be used as a quenching bath in which 80 the metal can be immediately immersed after heat-treatment. The use of such solution as a quenching bath for either tarnished or untarnished metal, is of particular importance in connection with heat-treating salt baths of the 85 kind above referred to, and more especially in the production of heated treated metals having a bright surface finish. Thus by means of the present invention, a continuous process is possible in which the heated metal is passed directly 90 and immediately from the heat treatment medium into the ammonium formate solution. A properly heat treated product having a bright or lustrous surface finish is obtained.

Another advantageous feature of my present 95 invention resides in the fact that after the metal is removed from the ammonium formate solution, by the evaporation of the vaporizable parts of the solution and the action of the solution on the metal, the wet solution or the residue after 100 the volatile components of the solution have evaporated adhering to the metal, has a greater affinity for oxygen than has the metal, so that the metal does not tarnish.

From the foregoing description, it is believed 105 that the particular novel features of my present disclosure and the advantages thereof in practical use or operation will be clearly and fully understood. While I have herein referred to a certain definite formula for the ammonium for-

mate solution and have stated the relative proportions of its constituent components, it is, of course, understood that these stated proportions are given for the preferred form, and that more or less variation thereof is permissible without noticeable disadvantageous effect in the results obtained in the use comprising my invention. And the residue of essentially sodium carbonate on the bright finish metals may be modified in use as a skin or film coating. Accordingly, the privilege is reserved of resorting to all such legitimate changes in the details of the present disclosure as may be fairly comprehended within the spirit and scope of the appended claims.

15 I claim:—

1. A scavenging solution for removing scale, oxide and other blemishes from the surfaces of metals, said solution containing sodium carbonate and ammonium formate.
- 20 2. A solution for removing scale, oxide and other blemishes from metal surfaces comprising a mixture of water and substantially equivalent parts of ammonium carbonate and sodium formate.
- 25 3. A solution for removing scale, oxide and other blemishes from metal surfaces comprising a mixture of the following named components in substantially the proportions stated: water 100 pounds, ammonium carbonate 4.1 lbs. and sodium formate 5.9 lbs.
- 30 4. In the removing of scale, rust, oxides, tarnish and other surface blemishes from metal surfaces, the process which comprises subjecting the surface of a metal having such a surface blemish to the action of a solution comprising ammonium formate for a time sufficient to remove the said surface blemish.
- 45 5. The process of producing a lasting bright finish on a metal surface subject to scaling, rusting, oxidizing and tarnishing which comprises dipping such a metal surface into a solution comprising ammonium formate until the said metal surface is brightened, followed by drying the surface without removal of salt residues.
- 50 6. In the process of producing bright surfaces upon heat treated metals having surfaces subject

to scaling, rusting, oxidizing and tarnishing, the step which comprises subjecting such a heat treated metal to the action of a solution comprising ammonium formate until said metal surface is brightened.

80 7. In the process of producing bright surfaces upon heat treated metals having surfaces subject to scaling, rusting, oxidizing and tarnishing, the process which comprises heat treating a metal in the usual manner in a salt bath, then quenching the heat treated metal in a solution containing ammonium formate.

85 8. The process of brightening the surface of a metal subject to scaling, rusting, oxidizing and tarnishing which comprises a simple dipping of the metal into a bath containing ammonium formate in solution, followed by immediate drying in such manner as to leave a surface film of residues on said metal.

90 9. In the production of bright finishes on metals subject to scaling, rusting, oxidizing and tarnishing, the process which comprises subjecting a metal surface to the action of a bath containing a hot solution of ammonium formate.

95 10. In the production of bright finishes on metals having surfaces subject to scaling, rusting, oxidizing and tarnishing, the process which comprises subjecting a metal surface to the action of a bath containing a solution of ammonium formate and sodium carbonate.

100 11. In the production of bright finishes on metals having surfaces subject to scaling, rusting, oxidizing and tarnishing, the process which comprises subjecting a metal surface to the action of a bath containing a solution formed by dissolving in water ammonium carbonate and sodium formate.

110 12. In the production of bright finishes on metals having surfaces subject to scaling, rusting, oxidizing and tarnishing, the process which comprises subjecting a metal surface to the action of a bath containing a solution formed by dissolving in 100 pounds of water, ammonium carbonate, 4.1 pounds and sodium formate 5.9 pounds, approximately.

120 ARTHUR E. BELLIS.

50

125

55

130

60

135

65

140

70

145

75

150